



US006559097B2

(12) **United States Patent**  
Mathiapanam et al.

(10) **Patent No.:** **US 6,559,097 B2**  
(45) **Date of Patent:** **May 6, 2003**

(54) **THERMALLY-RESPONSIVE RECORD MATERIAL**

(75) Inventors: **Ponnampalam Mathiapanam, Appleton, WI (US); Mark Robert Fisher, Appleton, WI (US); John Charles DeBraal, Appleton, WI (US)**

(73) Assignee: **Appleton Papers Inc., Appleton, WI (US)**

(\*) Notice: Subject to any disclaimer, the term of this patent is extended or adjusted under 35 U.S.C. 154(b) by 80 days.

(21) Appl. No.: **09/950,194**

(22) Filed: **Sep. 10, 2001**

(65) **Prior Publication Data**

US 2002/0049138 A1 Apr. 25, 2002

**Related U.S. Application Data**

(63) Continuation-in-part of application No. 09/391,575, filed on Sep. 8, 1999, now abandoned.

(51) **Int. Cl. 7** ..... **B41M 5/30**

(52) **U.S. Cl.** ..... **503/208; 503/209; 503/221**

(58) **Field of Search** ..... **503/208, 209, 503/221**

(56) **References Cited**

**U.S. PATENT DOCUMENTS**

|             |         |                      |         |
|-------------|---------|----------------------|---------|
| 4,531,140 A | 7/1985  | Suzuki et al. ....   | 346/209 |
| 4,628,335 A | 12/1986 | Igarashi et al. .... | 346/208 |
| 4,659,643 A | 4/1987  | Ishida et al. ....   | 430/157 |
| 4,855,278 A | 8/1989  | Igarashi et al. .... | 503/208 |
| 4,882,311 A | 11/1989 | Ikeda et al. ....    | 503/208 |
| 4,888,321 A | 12/1989 | Kawakami et al. .... | 503/208 |
| 4,980,336 A | 12/1990 | Akutsu et al. ....   | 503/209 |
| 4,981,835 A | 1/1991  | Iwakura et al. ....  | 503/209 |
| 4,985,391 A | 1/1991  | Ikeda et al. ....    | 503/208 |
| 5,041,604 A | 8/1991  | Saito et al. ....    | 558/415 |
| 5,081,099 A | 1/1992  | Akutsu et al. ....   | 503/209 |
| 5,143,890 A | 9/1992  | Tsuchida et al. .... | 503/201 |
| 5,179,068 A | 1/1993  | Goto ....            | 503/209 |
| 5,242,884 A | 9/1993  | Mando et al. ....    | 503/209 |
| 5,260,253 A | 11/1993 | Kawakami et al. .... | 503/216 |
| 5,312,950 A | 5/1994  | Boaz ....            | 558/51  |
| 5,563,017 A | 10/1996 | Yabuki et al. ....   | 430/138 |

**FOREIGN PATENT DOCUMENTS**

DE 3531125 C2 3/1986

|    |             |         |
|----|-------------|---------|
| EP | 0414243 A2  | 2/1991  |
| GB | 2165953 A   | 4/1986  |
| JP | 62-32329031 | 12/1987 |
| JP | 63-64787    | 3/1988  |
| JP | 2-134287    | 5/1988  |
| JP | 63-142381   | 6/1988  |
| JP | 1-168489    | 7/1989  |
| JP | 1-191962    | 7/1989  |

*Primary Examiner*—Bruce H. Hess

(74) *Attorney, Agent, or Firm*—Benjamin Mielius

(57) **ABSTRACT**

The present invention is a novel thermally-responsive record material comprising a substrate having provided thereon in substantially contiguous relationship an electron donating dye precursor, an acidic developer material, a compound of the formula



wherein  $\text{R}_1$ ,  $\text{R}_2$  and  $\text{R}_3$  are independently selected from hydrogen, alkyl, alkoxy, aryl, aralkyl, aralkoxy, halogen, alkoxyalkoxy, and aralkoxyalkoxy; with the proviso that when  $\text{R}_1$ ,  $\text{R}_2$  and  $\text{R}_3$  are hydrogen, that  $\text{R}_4$  is not benzyloxyethoxy or alkyl-substituted benzyloxyethoxy; wherein  $\text{R}_4$  is independently selected from alkoxyalkyl, alkoxyalkoxy, and aralkoxyalkoxy, and a suitable binder therefor.

In the context of the present invention the alkyl moieties in the alkyl, aralkyl, aralkoxy, alkoxyalkyl, alkoxyalkoxy and aralkoxyalkoxy preferably are eight carbons or less, and more preferably from one through four carbons. Substituents on aryl moieties in aryl, aralkyl, aralkoxy, and aralkoxyalkoxy groups can include hydrogen, alkyl, alkoxy and halogen. The alkyl group in these substituents also is eight carbons or less, and more preferably from one through four carbons.

The thermally responsive record material of the invention has the unexpected and remarkable properties of enhanced image intensity or density, and/or improved thermal response.

**14 Claims, No Drawings**

## THERMALLY-RESPONSIVE RECORD MATERIAL

This application under 35 USC §111(a) is a continuation-in-part and claims benefit per 35 USC §120 to U.S. Ser. No. 09/391,575 filed Sep. 8, 1999, now abandoned.

## BACKGROUND OF THE INVENTION

## 1. Field of the Invention

This invention relates to thermally-responsive record material. It more particularly relates to such record material in the form of sheets or rolls coated with color-forming material comprising chromogenic material (electron-donating dye precursor) and acidic color developer material. This invention particularly concerns a thermally-responsive record material (thermal record material) capable of forming a non-reversible image resistant to fade or erasure. The invention teaches record materials having improved thermal response, image formation, image retention and/or image density.

## 2. Description of Related Art

Thermally-responsive record material systems are well known in the art and are described in many patents, for example U.S. Pat. Nos. 3,539,375; 3,674,535; 3,746,675; 4,151,748; 4,181,771; 4,246,318; and 4,470,057 which are hereby incorporated by reference. In these systems, basic chromogenic material and acidic color developer material are contained in a coating on a substrate which, when heated to a suitable temperature, melts or softens to permit the said materials to react, thereby producing a colored mark.

Thermally-responsive record materials have characteristic thermal responses, desirably producing a colored image upon selective thermal exposure.

In the field of thermally-responsive record material, thermal response is defined as the temperature at which a thermally-responsive material produces a colored image of sufficient intensity or density. The desired temperature of imaging varies with type of application of the thermally-responsive product and the equipment used in the imaging process. The ability to shift the temperature at which thermal image of sufficient intensity or density is produced for any given combination of chromogenic material and developer materials is a much sought after and very valuable feature. For example, recent advances in high speed text or image recording demand both high speed recording devices and corresponding thermally-responsive recording materials with sufficient thermal response that are capable of producing a high intensity or high density color image at low thermal energy.

Also, in the field of thermally-responsive record material, the ability to increase the efficiency of the thermal image formation process has decided advantages. First among these is the ability to obtain the same image intensity or density with lower amount of reactants or, alternatively, to obtain a more intense image with the same amount of reactants.

It is an object of this invention to provide a thermally-responsive material having enhanced image intensity or density and/or improved thermal response.

## DETAILED DESCRIPTION

The present invention is a novel thermally-responsive record material comprising a support having provided thereon in substantially contiguous relationship an electron-donating dye precursor, an acidic developer material, a

compound of the formula



Wherein R<sub>1</sub>, R<sub>2</sub> and R<sub>3</sub> are independently selected from hydrogen, alkyl, alkoxy, aryl, aralkyl, aralkoxy, halogen, alkoxyalkoxy, and aralkoxyalkoxy

Wherein R<sub>4</sub> is independently selected from alkoxyalkyl, and aralkoxyalkoxy and a suitable binder therefor,

With the proviso that when R<sub>1</sub>, R<sub>2</sub> and R<sub>3</sub> are hydrogen, that R<sub>4</sub> then is not benzyloxyethoxy or alkyl-substituted benzyloxyethoxy.

In the context of the present invention the alkyl moieties in the alkyl, aralkyl, aralkoxy, alkoxyalkyl, alkoxyalkoxy and aralkoxyalkoxy preferably are each independently eight carbons or less, and more preferably of from one through four carbons. Substituents on aryl moieties in aryl, aralkyl, aralkoxy, and aralkoxyalkoxy groups can each independently include hydrogen, alkyl, alkoxy and halogen. The alkyl group in these substituents also is each independently eight carbons or less, and more preferably of from one through four carbons.

The thermally responsive record material of the invention has the unexpected and remarkable properties of enhanced image intensity or density, and/or improved thermal response. The compounds disclosed herein as formula I desirably function as sensitizers or modifiers facilitating reaction between the mark forming components yielding a more intense image at lowered temperatures or faster imaging.

Compounds illustrative of the invention according to formula I include without limitation:



3

-continued



4

-continued

C

I



D

Preferably, the thermally-responsive record material, 15 according to the invention comprises a support having provided thereon in substantially contiguous relationship an electron donating dye precursor, an acidic developer material, a compound of the formula



20

E

25



30

wherein R<sub>1</sub> and R<sub>2</sub> are each independently selected from hydrogen, alkyl, alkoxy, aryl, aralkyl, aralkoxy, halogen, alkoxyalkoxy and aralkoxyalkoxy, wherein R<sub>3</sub> is independently selected from hydrogen and alkyl, wherein R<sub>6</sub> is independently selected from aralkyl, said alkyl moieties each independently being from one to eight carbons, with the proviso that when R<sub>1</sub>, R<sub>2</sub> and R<sub>3</sub> are hydrogen, that R<sub>6</sub> is not benzyl or alkyl-substituted benzyl, and a suitable binder therefor. Additionally, the aryl moiety in each of the above groups each independently can be unsubstituted or substituted with alkyl (C<sub>1</sub>–C<sub>8</sub>), alkoxy (C<sub>1</sub>–C<sub>8</sub>) or halogen.

35

40

Optionally, the thermally-responsive record material according to the invention comprises a support having provided thereon in substantially contiguous relationship an electron donating dye precursor, an acidic developer material, a compound of the formula

(III)



50

55



H

Wherein R<sub>1</sub> and R<sub>3</sub> are each independently selected from hydrogen, halogen, alkyl, alkoxy, aryl, aralkyl, aralkoxy and aralkoxyalkoxy, wherein R<sub>6</sub> and R<sub>7</sub> are each independently selected from alkyl, and aralkyl, wherein each alkyl moiety herein is from one to eight carbons; wherein each aryl moiety herein is unsubstituted or substituted with alkyl (C<sub>1</sub>–C<sub>8</sub>), alkoxy (C<sub>1</sub>–C<sub>8</sub>), and a suitable binder therefor.

65

In general, the compounds according formulas I, II or III can be synthesized from a corresponding substituted or unsubstituted benzyloxyalkanol or alkoxyalkanol.

H



H



The alcohol is first converted to tosylate using p-toluenesulfonyl chloride (TsCl) and aqueous sodium hydroxide in acetonitrile, keeping the temperature of the reaction mixture below about 55° C. by slow addition of the base. Then, the tosylate is reacted with the corresponding phenol at 80° C. for about five hours to give the final product.

The times and the temperatures in this general protocol are approximate, and the person skilled in the art can readily adjust the reaction conditions, depending on the moieties involved, to obtain the desired product.

More specific and illustrative processes for the specific compounds, according to formulas I, II and III are set forth in more detail in synthesis example 1 and synthesis example 2.

In the heat sensitive record material according to the invention, the compound according to formulas I, II or III is preferably used in an amount corresponding to 10 to 1000 parts by weight per 100 parts of the electron donating dye precursor though when blended with other sensitizers, the amount of the compound according to formulas I, II or III can optionally be used in reduced amounts.

The record material includes a substrate or support material which is generally in sheet form. For purposes of this invention, sheets can be referred to as support members and are understood to also mean webs, ribbons, tapes, belts, films, cards and the like. Sheets denote articles having two large surface dimensions and a comparatively small thickness dimension. The substrate or support material can be opaque, transparent or translucent and could, itself, be colored or not. The material can be fibrous including, for example, paper and filamentous synthetic materials. It can be a film including, for example, cellophane and synthetic polymeric sheets cast, extruded, or otherwise formed. The gist of this invention resides in the color-forming composition coated on the substrate. The kind or type of substrate material is not critical.

The components of the color-forming system are in substantially a contiguous relationship, substantially homogeneously distributed throughout the coated layer or layers of material deposited on the substrate.

The term substantially contiguous relationship is understood to mean that the color-forming components are posi-

tioned in sufficient proximity such that upon melting, softening or subliming one or more of the components, a reactive color forming contact between the components is achieved. As is readily apparent to the person of ordinary skill in this art, these reactive components accordingly can be in the same coated layer or layers, or isolated or positioned in separate layers. In other words, one component can be positioned in the first layer, and reactive or sensitizer components or the ether compound according to Formulas I, II or III, or the acidic developer positioned in a subsequent layer or layers. The coating can optionally be applied to all of the substrate or spot printed on a certain portion. All such arrangements are understood herein as being substantially contiguous.

In manufacturing the record material, a coating composition is prepared which includes a fine dispersion of the components of the color-forming system, polymeric binder material, surface active agents and other additives in an aqueous coating medium. The composition can additionally contain inert pigments, such as clay, talc, aluminum hydroxide, calcined kaolin clay and calcium carbonate; synthetic pigments, such as urea-formaldehyde resin pigments; natural waxes such as Carnuba wax; synthetic waxes; lubricants such as zinc stearate; wetting agents; defoamers, and antioxidants. Other sensitizers can also be included. These sensitizers for example, can include acetoacetyl-*o*-toluidide, phenyl-1-hydroxy-2-naphthoate, 1,2-diphenoxylethane, and p-benzylbiphenyl. Optionally, the record material can be topcoated or use subcoats such as insulating layers or hollow spheres.

The color-forming system components are substantially insoluble in the dispersion vehicle (preferably water) and are ground to an individual average particle size of between about 1 micron to about 10 microns, preferably about 1–3 microns. The polymeric binder material is substantially vehicle soluble although latexes are also eligible in some instances. Preferred water soluble binders include polyvinyl alcohol, hydroxyethylcellulose, methylcellulose, methyl (hydroxypropyl)cellulose, starch, modified starches, gelatin and the like. Eligible latex materials include polyacrylates, styrene-butadiene-rubber latexes, polyvinylacetates, polystyrene, and the like. The polymeric binder is used to protect the coated materials from brushing and handling forces occasioned by storage and use of thermal sheets. Binder should be present in an amount to afford such protection and in an amount less than will interfere with achieving reactive contact between color-forming reactive materials.

Coating weights can effectively be about 3 to about 9 grams per square meter (gsm) and preferably about 5 to about 6 gsm. The practical amount of color-forming materials is controlled by economic considerations, functional parameters and desired handling characteristics of the coated sheets.

Eligible electron-donating dye precursors (or chromogenic compounds), include chromogens such as the phthalide, leucauramine and fluoran compounds. These chromogenic materials or electron donating dye precursors are well known color-forming compounds for use in color-forming record systems. Examples of the 5 compounds include Crystal Violet Lactone (3,3-bis(4-dimethylaminophenyl)-6-dimethylaminophthalide, U.S. Pat. No. RE 23,024); phenyl-, indolyl, pyrrolyl, and carbazolyl-substituted phthalides (for example, in U.S. Pat. Nos. 3,491,111; 3,491,112; 3,491,116; 3,509,174); nitro-, amino-, amido-, sulfonamido-, aminobenzylidene-, halo-, anilino-substituted fluorans (for example, the U.S. Pat. Nos. 3,624,107; 3,627,78; 3,641,011;

3,642,828; 3,681,390); spirodipyrans (U.S. Pat. No. 3,971,808); and pyridine and pyrazine compounds (for example, in U.S. Pat. Nos. 3,775,424 and 3,853,869). Other specifically eligible chromogenic compounds, not limiting the invention in any way, are: 3-diethylamino-6-methyl-7-anilino-flouran (U.S. Pat. No. 4,510,513); 3-dibutylamino-6-methyl-7-anilino-flouran; 3-dibutylamino-7-(2-chloroanilino) fluoran; 3-(N-ethyl-N-tetrahydrofurfuryl amino)-6-methyl-7-3',5'-tris(dimethylamino)spiro[9H-fluorene-9,1'(3'H)-isobenzofuran]-3'-one; 7-(1-ethyl-2-methyl indole-3-yl)-7-(4-diethylamino-2-ethoxyphenyl)-5,7-dihydrofuro[3,4-b]pyridin-5-one (U.S. Pat. No. 4,246,318); 3-diethylamino-7-(2-chloroanilino) fluoran (U.S. Pat. No. 3,920,510); 3-(N-methylcyclohexylamino)-6-methyl-7-anilinofluoran (U.S. Pat. No. 3,959,571); 7-(1-octyl-2-methylindole-3-yl)-7-(4-diethylamino-2-ethoxyphenyl)-5,7-dihydrofuro[3,4-b]pyridin-5-one; 3-diethylamino-7,8-benzofluoran; 3,3-bis(1-ethyl-2-methylindole-3-yl)phthalide; 3-diethylamino-7-anilinofluoran; 3-diethylamino-7-benzylaminofluoran; 3'-phenyl-7-dibenzylamino-2,2'-spirodi-[2H-1-benzopyran] and mixtures of any of the following.

Examples of eligible acidic developer material include the compounds listed in U.S. Pat. No. 3,539,375 as phenolic reactive material, particularly the monophenols and diphenols. Eligible acidic developer material also includes, without being considered as limiting, the following compounds which may be used individually or in mixtures: 4,4'-isopropylidinediphenol (Bisphenol A); p-hydroxybenzaldehyde; p-hydroxybenzophenone; p-hydroxypropiophenone; 2,4-dihydroxybenzophenone; 1,1-bis(4-hydroxyphenyl)cyclohexane; salicylanilide; 4-hydroxy-2-methylacetophenone; 2-acetylbenzoic acid; m-hydroxyacetanilide; p-hydroxyacetanilide; 2,4-dihydroxyacetophenone; 4-hydroxy-4'-methylbenzophenone; 4,4'-dihydroxybenzophenone; 2,2-bis(4-hydroxyphenyl)-4-methylpentane; benzyl(4-hydroxyphenyl)ketone; 2,2-bis(4-hydroxyphenyl)-5-methylhexane; ethyl-4,4-bis(4-hydroxyphenyl) pentanoate; isopropyl-4,4-bis(4-hydroxyphenyl) pentanoate; methyl-4,4-bis(4-hydroxyphenyl) pentanoate; alkyl-4,4-bis(4-hydroxyphenyl) pentanoate; 3,3-bis(4-hydroxyphenyl) pentane; 4,4-bis(4-hydroxyphenyl) heptane; 2,2-bis(4-hydroxyphenyl)-1-phenylpropane; 2,2-bis(4-hydroxyphenyl) butane; 2,2'-methylene-bis(4-ethyl-6-tertiarybutyl phenol); 4-hydroxycoumarin; 7-hydroxy-4-methylcoumarin; 2,2'-methylene-bis(4-octyl phenol); 4,4'-sulfonylidiphenol; 4,4'-thiobis(6-tertiarybutyl-m-cresol); methyl-p-hydroxybenzoate; n-propyl-p-hydroxybenzoate; benzyl-p-hydroxybenzoate. Preferred among these are the phenolic developer compounds. More preferred among the phenol compounds are 4,4'-isopropylidinediphenol, ethyl-4,4-bis(4-hydroxyphenyl)-pentanoate, n-propyl-4,4-bis(4-hydroxyphenyl)pentanoate, isopropyl-4,4-bis(4-hydroxyphenyl) pentanoate, methyl 4,4-bis(4-hydroxyphenyl) pentanoate, 2,2-bis(4-hydroxyphenyl)-4-methylpentane, p-hydroxybenzophenone, 2,4-dihydroxybenzophenone, 1,1-bis(4-hydroxyphenyl)cyclohexane, and benzyl-p-hydroxybenzoate. Acid compounds of other kind and types are eligible.

Examples of such other compounds are zeolites, phenolic novolak resins which are the product of reaction between, for example, formaldehyde and a phenol such as an alkylphenol, e.g., p-octylphenol, or other phenols such as p-phenylphenol, and the like; and acid mineral materials including colloidal silica, kaolin, bentonite, attapulgite, hallosyte, and the like. Some of the polymers and minerals do not melt but undergo color reaction on fusion of the chromogen.

The following examples are given to illustrate some of the features of the present and should not be considered as limiting. In these examples all parts or proportions are by weight and all measurement are in the metric system, unless otherwise stated.

In all examples illustrated the present invention a dispersion of a particular system component was prepared by milling the component in an aqueous solution of the binder until a particle size of between about 1 micron and 10 microns was achieved. The milling was accomplished in an attritor or other suitable milling device. The desired average particle size was about 1-3 microns in each dispersion.

Although some of the examples illustrate the invention using 2,2-bis(4-hydroxyphenyl)-4-methylpentane as the acidic developer material, the invention is readily practiced using any of the eligible acidic developer materials listed above.

The thermally-responsive sheets were made by making separate dispersions of chromogenic material, acidic material and the compound of formula I. The dispersions were mixed in the desired ratios and applied to a support with a wire wound rod and dried. Other materials such as fillers, antioxidants, lubricants and waxes can be added if desired. The sheets may be calendered to improve smoothness.

The thermal images are measured using a McBeth RD-922 densitometer. The densitometer is calibrated such that 0.08 indicates pure white and 1.79 a fully saturated black image.

Dispersions can be prepared in a quickie mill, attritor and small media mill. Optionally, but preferably dispersants can be added such as Nopco NDW at about 0.1 parts. This material is a sulfonated castor oil produced by Nopco Chemical Company. Surfynol 104 which is a di-tertiary acetylene glycol surface active agent produced by Air Products and Chemicals, Inc. could also be included, for example at about 0.4 parts. Additionally, water-soluble polymers other than polyvinyl alcohol (PVA) may be used to prepare the dispersions.

#### Description of the Preferred Embodiments

In the following examples, general procedures for preparing certain compounds listed above are described; the examples are not intended to be exhaustive and the moieties, as previously defined, are all eligible for use in any combination in preparing the compounds. Unless otherwise noted, all measurements, percentages and parts are by weight.

#### SYNTHESIS EXAMPLE 1

##### Preparation of 2-(4-chlorobenzyl)ethyl-(4-phenyl)phenyl Ether (Compound A)

4-Phenylphenol (34.0 g, 0.2 mole), ethylene carbonate (20.0 g, 0.227 mole) and tetrabutylammonium bromide (6.5 g, 0.02 mole) were heated to 155° C. with stirring in a three-necked, round-bottom flask equipped with a mechanical stirrer and a reflux condenser. After 5 hours, the reaction mixture was cooled to 110° C., most of the lower boiling materials were removed under reduced pressure. Finely powdered potassium hydroxide (17.0 g, 0.3 mole) was added and the reaction mixture stirred for 5 minutes. Then, 4-chlorobenzyl chloride (35.0 g, 0.217 mole) was added and the reaction mixture was kept at 110° C. with vigorous stirring. After 4 hours, toluene (250 ml) was added and the reaction mixture was cooled to 60° C. Water (100 ml) was added and stirring continued. Toluene layer was separated and the aqueous layer was extracted twice with warm toluene. The toluene extracts were combined, washed with water, dried and concentrated. The residue was recrystall-

lized from toluene/methanol. Yield: 55.8 g (82%), white solid, M.P.: 85–87° C.

## SYNTHESIS EXAMPLE 2

## Preparation of [2-(Benzylxy)ethyl]-4-[4-(bromophenyl)]phenyl Ether (Compound B)

2-(Benzylxy)ethanol (30.5 g, 0.2 mole) and p-toluenesulfonyl chloride (40.0 g, 0.2 mole) were added with stirring to acetonitrile (100 ml) in a 500 ml, four-necked, round-bottom flask, equipped with a mechanical stirrer, reflux condenser, thermometer and a dropping funnel. Aqueous sodium hydroxide (17.0 g, 0.425 mole/35 ml of water) was added slowly from the dropping funnel while the temperature of the reaction mixture was kept below 55° C. After the addition was complete, the reaction mixture was stirred for one hour as it cooled to room temperature. Then 4-(4-bromophenyl)phenol (50.0 g, 0.2 mole) was added and the reaction mixture was warmed to 80° C. with vigorous stirring for 5 hours. The GC analysis of the reaction mixture (OV-1 column, 100° C. for 2 mins, 25° C./min to 300° C.) showed that the reaction was complete.

The reaction mixture was poured into ice/water mixture and stirred. The precipitated solid was filtered and washed with cold water, dried and dissolved in toluene. The toluene solution was washed with aqueous sodium hydroxide (10%) and water; dried and concentrated. The crude product was dissolved in toluene and the toluene solution was passed through a column of alumina using toluene as eluant. Fractions containing the product were collected, combined and concentrated. The residue was recrystallized from toluene/methanol. Yield: 58.7 g (77%), white solid, M.P.: 91–92° C.

-continued

| Components                                           | Parts |
|------------------------------------------------------|-------|
| Dispersion A - Chromogenic Material                  | 40    |
| Chromogenic Material                                 | 32.0  |
| Binder, 20% solution of Polyvinyl alcohol in water   | 27.4  |
| Defoaming and dispersing agents                      | 0.4   |
| Water                                                | 40.2  |
| Dispersion A1 - Chromogenic Material is ODB-2        | 45    |
| 3-Di-(n-butylamino)-6-methyl-7-anilinofluoran        |       |
| Dispersion A2 - Chromogenic Material is ETAC         |       |
| 3-(N-Ethyl-N-p-tolylamino)-6-methyl-7-anilinofluoran | 50    |
| Dispersion B - Acidic Material                       |       |
| Acidic material                                      | 42.5  |
| Binder, 20% solution of Polyvinyl alcohol in water   | 21.2  |
| Defoaming and dispersing agents                      | 36.1  |
| Dispersion B1 - Acidic Material is AP-5              | 55    |
| 2,2-Bis(4-hydroxyphenyl)-4-methylpentane             |       |
| Dispersion B2 - Acidic Material is TGSA              |       |
| Bis(3-allyl-4-hydroxyphenyl)sulfone                  | 60    |
| Dispersion C - Sensitizing Material                  |       |
| Sensitizing Material                                 | 42.5  |
| Binder, 20% solution of Polyvinyl alcohol in water   | 21.2  |
| Defoaming and dispersing agents                      | 0.2   |
| Water                                                | 36.1  |
| Dispersion C1 - Sensitizing Material is DMT          | 65    |
| Dimethyl Terephthalate                               |       |

-continued

| Components                                        | Parts | Example #      | McBeth intensity at 12.0 mJ/mm <sup>2</sup> | McBeth intensity at 31.8 mJ/mm <sup>2</sup> |
|---------------------------------------------------|-------|----------------|---------------------------------------------|---------------------------------------------|
| Dispersion A - Chromogenic Material               |       | 5              |                                             |                                             |
| <u>Comparative Example 7</u>                      |       | 1              | 0.48                                        | 1.34                                        |
| Coating Formulation 1 Using                       |       | 2              | 0.21                                        | 1.31                                        |
| Dispersion A1 (ODB-2)                             |       | 3              | 0.49                                        | 1.44                                        |
| Dispersion B2 (TGSA)                              |       | 4              | 0.23                                        | 1.27                                        |
| Dispersion C1 (DMT)                               |       | 10             | Comparative 1                               | 0.23                                        |
| <u>Comparative Example 8</u>                      |       | Comparative 2  | 0.10                                        | 1.30                                        |
| Coating Formulation 1 Using                       |       | Comparative 3  | 0.28                                        | 1.40                                        |
| Dispersion A2 (ETAC)                              |       | Comparative 4  | 0.11                                        | 1.01                                        |
| Dispersion B2 (TGSA)                              |       | Comparative 5  | 0.31                                        | 1.39                                        |
| Dispersion C1 (DMT)                               |       | Comparative 6  | 0.10                                        | 1.43                                        |
| <u>Comparative Example 9</u>                      |       | Comparative 7  | 0.44                                        | 1.43                                        |
| Coating Formulation 1 Using                       |       | Comparative 8  | 0.18                                        | 1.32                                        |
| Dispersion A1 (ODB-2)                             |       | Comparative 9  | 0.36                                        | 1.42                                        |
| Dispersion B2 (TGSA)                              |       | Comparative 10 | 0.27                                        | 1.33                                        |
| Dispersion C2 (pBBP)                              |       | Comparative 11 | 0.52                                        | 1.43                                        |
| <u>Comparative Example 10</u>                     |       | Comparative 12 | 0.17                                        | 1.14                                        |
| Coating Formulation 1 Using                       |       | Comparative 13 | 0.20                                        | 1.28                                        |
| Dispersion A2 (ETAC)                              |       | Comparative 14 | 0.11                                        | 0.96                                        |
| Dispersion B2 (TGSA)                              |       | Comparative 15 | 0.32                                        | 1.36                                        |
| Dispersion C2 (pBBP)                              |       | Comparative 16 | 0.11                                        | 0.83                                        |
| <u>Comparative Example 11</u>                     |       |                |                                             |                                             |
| Coating Formulation 1 Using                       |       |                |                                             |                                             |
| Dispersion A1 (ODB-2)                             |       |                |                                             |                                             |
| Dispersion B2 (TGSA)                              |       |                |                                             |                                             |
| Dispersion C3 (stearamide wax)                    |       |                |                                             |                                             |
| <u>Comparative Example 12</u>                     |       |                |                                             |                                             |
| Coating Formulation 1 Using                       |       |                |                                             |                                             |
| Dispersion A2 (ETAC)                              |       |                |                                             |                                             |
| Dispersion B2 (TGSA)                              |       |                |                                             |                                             |
| Dispersion C3 (stearamide wax)                    |       |                |                                             |                                             |
| Coating Formulation 2                             |       |                |                                             |                                             |
| <u>Comparative Example 13</u>                     |       |                |                                             |                                             |
| Dispersion A (Chromogenic)                        | 7.6   |                |                                             |                                             |
| Dispersion B (Acidic)                             | 15.0  |                |                                             |                                             |
| Dispersion C (Sensitizing)                        | 0.0   |                |                                             |                                             |
| Binder, 10% solution of polyvinylalcohol in water | 45.5  |                |                                             |                                             |
| Filler slurry, 50% in water                       | 19.0  |                |                                             |                                             |
| <u>Comparative Example 14</u>                     |       |                |                                             |                                             |
| Coating Formulation 2 Using                       |       |                |                                             |                                             |
| Dispersion A1 (ODB-2)                             |       |                |                                             |                                             |
| Dispersion B1 (AP-5)                              |       |                |                                             |                                             |
| <u>Comparative Example 14</u>                     |       |                |                                             |                                             |
| Coating Formulation 2 Using                       |       |                |                                             |                                             |
| Dispersion A2 (ETAC)                              |       |                |                                             |                                             |
| Dispersion B1 (AP-5)                              |       |                |                                             |                                             |
| <u>Comparative Example 15</u>                     |       |                |                                             |                                             |
| Coating Formulation 2 Using                       |       |                |                                             |                                             |
| Dispersion A1 (ODB-2)                             |       |                |                                             |                                             |
| Dispersion B2 (TGSA)                              |       |                |                                             |                                             |
| <u>Comparative Example 16</u>                     |       |                |                                             |                                             |
| Coating Formulation 2 Using                       |       |                |                                             |                                             |
| Dispersion A2 (ETAC)                              |       |                |                                             |                                             |
| Dispersion B2 (TGSA)                              |       |                |                                             |                                             |

The examples were coated at 3.0 gm/m<sup>2</sup>. A topcoat was applied at 3.5 gm/m<sup>2</sup>. The examples were then printed on the ATLANTEK model 300. The optical density was measured using a McBeth II densitometer. The results are in the following chart.

25 The principles, preferred embodiments, and modes of preparation the present invention have been described in the foregoing specification. The invention which is intended to be protected herein, however, is not to be construed as 30 limited to the particular forms disclosed, since these are to be regarded as illustrative rather than restrictive. Variations and changes can be made by those skilled in the art without departing from the spirit and scope of the invention.

35 We claim:

1. A thermally-responsive record material comprising a substrate having provided thereon in substantially contiguous relationship an electron donating dye precursor, an 40 acidic developer material, a compound of the formula:



50 wherein R<sub>1</sub>, R<sub>2</sub>, and R<sub>3</sub> are each independently selected from hydrogen, alkyl, alkoxy, aryl, aralkyl, aralkoxy, halogen, alkoxyalkoxy and aralkoxyalkoxy,

55 wherein R<sub>4</sub> is independently selected from alkoxyalkyl and aralkoxyalkoxy,

with the proviso that when R<sub>1</sub>, R<sub>2</sub> and R<sub>3</sub> are hydrogen, that R<sub>4</sub> is not benzyloxyethoxy or alkyl-substituted benzyloxyethoxy,

60 said alkyl moieties each independently being from one to eight carbons, said aryl moieties each independently being unsubstituted or substituted by alkyl ((C<sub>1</sub>-C<sub>8</sub>)), alkoxy (C<sub>1</sub>-C<sub>8</sub>) or halogen,

and a suitable binder therefor.

2. The thermally-responsive record material according to claim 1 wherein the compound according to formula I is

13



3. The thermally-responsive record material according to claim 1 wherein the compound according to formula I is



4. The thermally-responsive record material according to claim 1 wherein the compound according to formula I is



5. The thermally-responsive record material according to claim 1 wherein the compound according to formula I is used in an amount of from 10 to 1000 parts by weight per 100 parts of the electron donating dye precursor.

6. The thermally-responsive record material according to claim 1 wherein the electron donating dye precursor is a fluoran compound.

7. A thermally-responsive record material comprising a substrate having provided thereon in substantially contiguous relationship an electron donating dye precursor, an acidic developer material, a compound of the formula



wherein R<sub>1</sub> and R<sub>2</sub> are each independently selected from alkyl, alkoxy, aryl, aralkyl, aralkoxy, halogen, alkoxy-alkoxy and an alkoxyalkoxy,  
wherein R<sub>3</sub> is independently selected from hydrogen and alkyl,  
wherein R<sub>6</sub> is independently selected from aralkyl,

14

said alkyl moieties each independently being from one to eight carbons,  
with the proviso that when R<sub>1</sub>, R<sub>2</sub> and R<sub>3</sub> are hydrogen, that R<sub>6</sub> is not benzyl or alkyl-substituted benzyl,  
said aryl moieties each independently being unsubstituted or substituted by alkyl (C<sub>1</sub>–C<sub>8</sub>), alkoxy (C<sub>1</sub>–C<sub>8</sub>) or halogen,  
and a suitable binder therefor.

8. The thermally-responsive record material according to claim 7, wherein the compound according to formula II is



9. The thermally-responsive record material according to claim 7, wherein the compound according to formula II is



10. The thermally-responsive record material according to claim 7, wherein the compound according to formula II is



11. A thermally-responsive record material comprising a substrate having provided thereon in substantially contiguous relationship an electron donating dye precursor, an acidic developer material, a compound of the formula



wherein R<sub>1</sub> and R<sub>3</sub> are each independently selected from hydrogen, halogen, alkyl, alkoxy, aryl, aralkyl, aralkoxy and aralkoxyalkoxy,  
wherein R<sub>6</sub> and R<sub>7</sub> are each independently selected from alkyl, and aralkyl,  
said alkyl moieties each independently being from one to eight carbons,

15

said aryl moieties each independently being unsubstituted or substituted by alkyl (C<sub>1</sub>–C<sub>8</sub>), alkoxy (C<sub>1</sub>–C<sub>8</sub>) or halogen,

and a suitable binder therefor.

12. The thermally-responsive record material according to claim 11 wherein the compound according to formula III is

16



<sup>10</sup> 14. The thermally-responsive record material according to claim 11 wherein the compound according to formula III is



13. The thermally-responsive record material according to claim 11 wherein the compound according to formula III is

\* \* \* \*